# EUROPEAN PATENT SPECIFICATION

(11) **EP 1 224 247 B1**
(45) Date of publication and mention of the grant of the patent: **07.02.2007**
(21) Application number: 00962686.2
(22) Date of filing: 15.09.2000
(51) Int. Cl.: C10L 1/06

(54) **FUEL COMPOSITIONS**
BRENNSTOFFZUSAMMENSETZUNGEN
COMPOSITIONS DE CARBURANT

(30) Priority: 23.09.1999 GB 9922553
(43) Date of publication of application: 24.07.2002
(73) Proprietor: BP OIL INTERNATIONAL LIMITED, Sunbury-on-Thames, Middlesex TW16 7BP (GB)
(72) Inventor: BUTLER, Graham, Churt, Surrey GU10 2HS (GB); CLARK, Alisdair Quentin, Aldershot, Hampshire GU12 6LS (GB)
(74) Representative: Perkins, Nicholas David
(86) International application number: PCT/GB2000/003569
(87) International publication number: WO 2001/021738

(56) References cited:
- EP-A- 0 994 088
- WO-A-00/77130
- WO-A-98/22556

## Description

This invention relates to a fuel composition, in particular a gasoline composition for transportation uses e.g. use in motor vehicles or aircraft.

For many years manufacturers of spark ignition combustion engines have been striving for higher efficiency to make optimum use of hydrocarbon based fuels. But such engines require gasolines of higher octane number, which has been achieved in particular by addition of organo lead additives, and latterly with the advent of unleaded gasolines, by addition of MTBE. But combustion of any gasoline gives rise to emissions in the exhaust gases, e.g. of carbon dioxide, carbon monoxide, nitrogen oxides (NOx) and toxic hydrocarbons and such emissions are undesirable.

Unleaded gasolines have been discovered having high Octane Number but producing low emissions on combustion.

The present invention provides a formulated unleaded gasoline as claimed in claim 1.

Unless otherwise stated all percentages in this specification are by volume, and disclosures of a number of ranges of amounts in the composition or gasoline for 2 or more ingredients includes disclosures of all sub-combinations of all the ranges with all the ingredients.

The compounds A are alkanes of 8-12 carbon atoms (especially 8 or 10 carbons) with at least 4 methyl and/or ethyl branches, e.g. 4-6 branches, preferably 4 or 5 or especially 4 branches. Methyl branches arc preferred. The compounds usually have their longest chain of carbon atoms, hereinafter called their backbone chain, with 4-7 e.g. 4-6 chain carbon atoms (especially 4 or 5) to which the methyl, and/or ethyl branches arc attached. Advantageously, especially in relation to the first to tenth groupings as described further below, there are no branched groups constituting the branches other than methyl or ethyl, and, in the backbone chain of carbon atoms, there are especially no linear alkyl groups of more than 2 carbons nor 1,2 ethylene or 1,3 propylene.groups in the chain, and especially no methylene groups in the chain except as part of an ethyl group; thus there are especially no n-propyl or n-butyl groups forming part of the backbone chain. Preferably there is at least one compound (A) alkane of 9-12 e.g. 9 or 10 carbons, and in this case there is usually less than 50% or 10% of an 8 carbon alkane compound e.g. with 3 methyl branches.

The compounds can have 1 or 2 methyl or ethyl groups attached to the same carbon atom of the backbone chain, especially 1 or 2 methyl groups and 0 or 1 ethyl groups. The carbon atom in the backbone at which the branching occurs is non-terminal i.e. is an internal carbon in the backbone chain, especially the 2, 3 and/or 4 numbered carbon in the backbone. Thus advantageously the compound has geminal methyl substituents on position 2, 3 or 4 carbon atoms, especially position 2, but in particular position 3.

In a first grouping of compounds A, there is at least one pair of geminal methyl branch substituents, and they are on position 2, or there are 2 or 3 pairs of geminal branches at least 2 pairs being on vicinal (ie adjacent) carbon atoms, as in a group - CMe₂-CMe₂-.

In a second grouping of the compounds A there are 1, 2 or 3 pairs of geminal methyl branch substituents on a 4-6 carbon chain backbone, and, if any Ethyl CMe₂-structure is present, then there are 2 Ethyl CMe₂ groups in the compound. The compounds of the second grouping advantageously have a MON value of at least 100.

In a third grouping of the compounds, there is one geminal methyl branch grouping i.e. -CMe₂- on the backbone, while on one or both of the adjacent carbon atoms of the backbone, there is/are one or two methyl or ethyl branches/especially I or 2 methyl branches.

In a fourth grouping of the compounds there are one, two or three pairs of geminal methyl branches. If there are 2 or 3 pairs then at least 2 pairs are on adjacent backbone carbon atoms, and if there is only one pair, then they are preferably on the 2 position backbone carbon and there is a methyl branch at least on the 3 position backbone carbon. Such compounds usually have a RON value of at least 111. Advantageously the compounds are of 8 or 10 carbon atoms.

In a fifth grouping the compound A has 2 or 3 pairs of geminal methyl branches at least 2 pairs being on adjacent backbone carbon atoms, and the compound has a symmetrical structure. Such compounds usually have RON value of at least 120, and especially are of 8 or 10 carbon atoms.

In a sixth grouping the compounds have a linear backbone chain of 4 or 6 carbons and have 4-6 e.g. 4, 5 or 6 especially 4 methyl branches, in at least one geminal group (CMe₂) especially in the absence of a 1,2 ethyl group in the backbone.

In a seventh grouping, the compounds have a linear backbone chain of 5 or 6 carbons and have 4-6 e.g. 4, 5 or 6 especially 4 branches in at least one geminal group, with the proviso that if there are 4 methyl branches and the compound contains an Ethyl CMe₂ group, then the compound contains two such Ethyl CMe₂ groups. Such compounds are usually liquid at 25°C and generally have a RON value of greater than 105. Especially there are only methyl branches; such compounds usually have a MON value of at least 101.

Advantageously in an eighth grouping the compounds A contain 1, 2 or 3 carbon atoms with geminal methyl branches, and if there is only one such carbon atom with geminal branches, then there is/are one or two branches on a vicinal carbon atom to the geminal one, and any ethyl -C- chain group in the backbone chain has 5 carbon atoms i.e. is (Ethyl)₂CH or Ethyl CMe₂-. Especially there are 2 or 3 vicinal carbon atoms in the backbone, each carrying 2 methyl branches.

A particularly preferred sub-class (ninth grouping) for the compound A is alkanes with alkyl substituents on vicinal internal carbon atoms, with a total of 4, 5 or 6 carbon atoms in said substituents.

Among this sub-class are preferred ones especially with geminal methyl groups on internal chain carbon atoms. Particularly preferred sub-class compounds A have 4 or 5 methyl substituents on the carbon backbone, especially with at least 2 on the same backbone carbon atom (in particular in two -CMe₂- groups) especially in a -CMe₂-CMe₂ group.

In another aspect of the invention there is provided an unleaded blend composition having a MON value of at least 81 or 85 and RON value of at least 91 or 94, which comprises component (a) a total of at least 10 or 15% of one or more branched alkane compounds A¹ of 8-12 carbons (especially with 4-7 or 4-6 backbone carbon atoms), with at least 4 methyl or ethyl branches and with at least 2 backbone carbon atoms which are secondary and/or tertiary carbon atoms, with the proviso that if there are only 2 such carbon atoms, then both are tertiary, there being a minimum of at least 1, 2, 5 or 10% (by volume of the composition) of at least one individual compound A¹, and component (b) of nature and in amount as described herein, with the preferred proviso as described above. In the above component A¹, which may be the same or different from A, there may thus in a tenth grouping be in the backbone internal (i.e. non-terminal) carbon atoms which are (i) 2 or 3 tertiary carbons, (ii) especially vicinal ones, or (iii) 2 tertiary and one sec. carbon or (iv) 2 tertiary and one or 2 primary carbon, or (iv) 1 or 2 tertiary and 1 or 2 sec subject to at least 4 branches, in particular (vi) with the tert and a sec. carbon vicinal and (vii) when there are 2 tert, these are vicinal or non-vicinal and (viii) with 1 or 2 vicinal tert and sec. carbons subject to at least 4 branches. The compounds A¹ usually are free from 2 primary internal backbone carbon atoms on vicinal carbons i.e. as in 1,2-ethylene group. Preferably any primary internal backbone carbon atoms are not between, e.g. adjacent on both sides to, a tert and/or sec, carbon on the one hand and a tert and/or sec. carbon on the other hand. Especially at least the said 2 backbone carbon atoms above in compounds A¹ are vicinal.

In another category, the eleventh grouping is of compounds A¹ which contain, with the proviso of at least 4 branched groups, (i) as at least one end of the backbone a group of formula CHR¹R² where each of R¹ and R², which are the same or different is a methyl or ethyl group or (ii) as at least one end of the backbone a group of formula CR¹R²R³ where R¹ and R² are as defined above and R³ is methyl or ethyl. Preferred are such compounds A¹ which have both (i) and (ii), especially when the CHR¹R² group is CHMe₂ when the compound has 8 carbons or a backbone of 5 carbons and when all internal carbon atoms in the backbone chain are secondary or tertiary.

The compounds A or A¹ may have a boiling point at 1 bar pressure of 150-175°C, 130-140°C, 110-129°C, or 90-109°C. In particular the boiling point is preferably at least 105°C e.g. 105-175°C, with the preferred proviso that it is at least 112°C such as 112-175°C unless the compound A or A¹ has 4 alkyl branches.

In another category the compounds A or A¹ may have 4-6 methyl and/or ethyl branches on a 4-7 or 4-6 carbon backbone, and especially a ratio of carbon atom in branches to carbon atoms in the backbone chain of at least 0.63:1 e.g. 0.63-1.6:1 such as 0.63-1.0:1. The compounds usually have 9 or 10 carbons, unless the above ratio is at least 0.63, 0.75 or 0.9.

Preferred compounds are 3344 tetramethyl hexane (A1), 2233 tetramethyl butane (A2), 2233 tetramethyl pentane (A7), 22334 pentamethyl pentane (A12) 22344 pentamethyl pentane (A13) 2334 tetramethyl pentane (A14) 2234 tetramethyl pentane (A15) 223344 hexamethyl pentane (A16) 22446 pentamethyl heptane. Of these (A1) and (A2) are most preferred with (A7) being also very valuable.

The compounds A and A¹ are either known compounds and may be made according to the published literature, or are novel and may be made by conventional methods known per se in the literature (e.g. as described in Kirk Othmer Encyclopaedia of Chemical Technology 3rd Ed. Publ. Wiley). Examples of suitable methods of preparation are known carbon-carbon coupling techniques for making alkanes. The technique may involve reactions of one or more usually 1 or 2 alkyl chlorides, bromides or iodides with an elemental metal of Group IA, IIA, IB or IIB of the Periodic Table in Advanced Inorganic Chemistry by F.A.Cotton + G.wilkinson, Pub. Interscience New York 2nd Ed. 1966, especially sodium, magnesium, or zinc. The alkyl halide is usually a branched chain one of 3-6 carbons, in particular with methyl or ethyl branches, and especially with the halogen atom attached to a CMe₂ group in at least one of the alkyl halides. Preferably the halide is of formula MeCMe₂X or EtCMe₂X, where X is Cl, B or 1, and the other halide, if any, is a tertiary alkyl halide or a secondary one e.g. of formula RR¹CHX, wherein at least one of R and R¹ is a branched alkyl group e.g. of 3-5 carbons such as isopropyl or t-butyl, and the other (if any) is methyl or ethyl or a primary branched alkyl halide e.g. of formula R¹¹CH₂X, where R¹¹ is a branched alkyl group 4-5 carbons with methyl or ethyl branches, such as isobutyl or isoamyl. Alternatively both halides can be secondary e.g. of formula RR¹CHX, as defined above and R^{III}R^{IV}CHX where R^{III} is methyl or ethyl and R^{IV} is as defined for R, such as isopropyl or one can be secondary (as above) and one can be primary e.g. methyl or ethyl halide. The methods of coupling optimum for any particular compound A or A¹ depend on availability of the precursor alkyl halide(s) so that in addition to the above kinds, coupling via methyl or ethyl halides with branched alkyl halides of 6-9 carbons may also be used e.g. pentamethyl ethyl bromide and methyl magnesium bromide to form A2. The alkyl halide(s) can react together in the presence of the metal (as in a Wurtz reaction with sodium), or one can react first with the metal to form an organometallic compound e.g. a Grignard reagent or organo zinc, followed by reaction of the organometallic with the other alkyl halide. If desired the Grignard reagent reaction can be in the presence of a metal of Group IB or IIB, such as silver, zinc or copper (especially high activity copper). If desired the Grignard reagent from one or both alkyl halides can be reacted with the latter metal to form other alkyl metallic species e.g. alkyl silver or alkyl copper compounds, which can disproportionate to the coupled alkane. The Grignard reagent(s) can also react with a cuprous halide to form alkyl copper species for disproportionation. Finally an organometallic compound, wherein the metal is of Group IA or IIA e.g. Li or Mg can be coupled by reaction with a cuprous complex to give a coupled alkane. Use of only I alkyl halide gives a symmetrical alkane, while use of a mixture of alkyl halides gives a mixture of alkanes, usually each of the symmetrical dimers and an unsymmetrical alkane formed from both alkyl halides.

The above organometallic reactions are usually conducted under inert conditions, i.e. anhydrous and in the absence of oxygen e.g. under dry nitrogen. They are usually performed in an inert solvent e.g. a dry hydrocarbon or ether. At the end of the reaction any residual organometallic material is decomposed by addition of a compound with active hydrogen e.g. water or an alcohol, and the alkanes are distilled off, either directly or after distribution between an organic and aqueous phase.

Examples of the above processes are the coupling of tertbutyl chloride in the presence of Mg and diethyl ether to form compound A(2) (as described by D.T.Flood et al, J.Amer Chem. Soc. 56, (1934) 1211, or R.E.Marker et al, J.Amer Chem. Soc. 60, (1938) 2598 or F.C.Whiteman et al, J.Amer Chem. Soc. 55, (1933) 380), and the corresponding coupling of EtCMe₂ halides to form compound A1. Other preparations of highly branched alkanes are described in M Tamura and J.Kochi, J.Amer. Chem. Soc. Vol.93, Part 6 (March 24, 1971) and F.O.Ginah et al, J. Org. Chem. Vol. 199, 55 pp584-589 and R.Y.Levina & V.K.Daukshas, Zhur.Obschei Khim. Vol. 29 (1959) and F L Howard etal, J Res. Nat. Bur. Standards Research Paper RP1779, Vol 38 March 1947 pp 365-395. The disclosures of these documents is incorporated herein by reference.

The crude alkanes made by the above processes, especially the symmetrical ones, may be used as such in the blends of the invention or may be purified further e.g. by distillation first. The crude unsymmetrical alkanes may be also purified, but are preferably used as such as the by-product alkanes are often useful hydrocarbons for the blend, e.g. coupling of t BuX and EtCMe₂X as described above produces a mixture of alkanes containing A1, A2 and A7.

Other known methods of making the alkanes A or A¹, are reaction of alkyl metallic compounds e.g. Grignard reagents with carbonyl compounds such as aldehydes, ketones, esters, or anhydrides to form branched chain carbinols, which are dehydrated to the corresponding olefin, which is hydrogenated to the alkane. Thus 2,2,3,4-tetra methyl pentane may be made from isopropyl magnesium bromide and methyl t-butyl ketone (followed by dehydration and hydrogenation),

Thus the present invention produces an unleaded blend composition of MON value at least 81 or 85 and RON value at least 91 or 94 which comprises (a) a total of at least 10 or 15% of one or more branched hydrocarbon compound A or A¹ there being a minimum of at least 1, 2 or 5% of at least one individual compound A or A¹ and (b) at least 20% of at least one different liquid hydrocarbon of bp60-160°C having a MON value of at least 70 and RON value at least 90 especially when (b) is not within the definition of A or A¹. Examples of the liquid hydrocarbons are paraffins, such as linear or branched chain alkanes of 4-8 carbons, such as isobutane, butane, isopentane, dimethyl alkanes such as 23 dimethyl butane, cycloalkanes, such as cyclopentane and cyclohexane, aromatics and olefins.

Another unleaded blend composition of the invention of MON value of at least 81 or 85 and RON value of at least 91 or 94 comprises component (a) as above and component (b) at least 20% of at least one of a straight run naphtha, alkylate isomerate (bp25-80°C) heavy reformate, light reformate (bp20-79°C), hydrocrackate, aviation alkylate (bp30-190°C), straight run gasoline, cracked spirit, such as heavy or light catalytic cracked spirit or steam cracked spirit. The straight run products are produced directly from crude oil by atmospheric distillation. The naphtha may be light naphtha of bp30-90°C or medium naphtha of bp90-150° or heavy naphtha of bp 150-220°C.

In the blends of the invention, the amount of at least one individual compounds A or A¹ is usually at least 1, 2 or 5%, or at least 10 or 15%, such as 5-60%, e.g. 15-60%, or 8-25%, 20-35% or 30-55% or 2-10%. The amount of 2,2,4-trimethyl pentane if present is usually at least 10% of the composition. Total amounts of trimethyl pentanes in the blend are preferable less than 69% of the blend, but advantageously at least 26% (especially when the amount of aromatics is less than 17%). If a 9 or 10 carbon alkane is (a), then the amount of 2,2,4-trimethyl pentane is especially less than 70 or 50%. More than one such compound A or A¹ may be present e.g. of higher and lower RON in weight ratios of 9:1 to 0.5:99.5, such as 0.5:1 to 5:1 or 5:95 to 20:80, particularly for mixtures of compounds A1 and A2 and/or with higher or lower boiling points (atmospheric pressure) e.g. those in which the compounds A and/or A¹ have boiling points differing by at least 10°C e.g. at least 40°C such as 10-70°C or 20-50°C the relative amounts being as described above. In the blends amounts of compounds A or A¹ of RON at least 138 e.g. A1 may be 1-40%, such as 2-10 or 20-35%, while those of compounds A or A¹ of RON 120-138 e.g. A2 may be 1-60, such as 5-60, 8-25 or 30-55% (especially when used with the higher RON compound) or 15-50% when used as sole compound A. Total amounts of all compounds A and A¹ (if any) in the blend are at least 10 or 15% such as 15-70 e.g. 15-60, 15-40 or 30-55% or 40-60% or 10-35%.

The blend may also comprise predominantly aliphatic refinery streams which are usually liquid e.g. at 20°C such as naphtha, straight run gasoline (also known as light naphtha bp 25-120°C), alkylate and isomerate. Amounts in total of these may be 10-70%, such as 10-30, 30-70 or 35-65%. Amounts of naphtha may be 0-70% or 1-70% such as 10-30, 30-70 or 35-65%, while amounts of light naphtha may be 0 or 1-70 such as 1-20 or especially 30-65%, and amounts of medium naphtha may be 0 or 1-55, such as 3-20 or 15-55%. The volume ratio of light to medium naphtha may be 50:1 to 1:50, such as 0.5-20:1 or 1:0.5-50. Amounts of alkylate or isomerate (if present) may be 0.5-20% such as 1-10%, while amounts of hydrocrackate may be 0.5-30% e.g. 10-30%. A preferred blend comprises 20-60% compound A or A¹ and conversely 80-40% straight run gasoline, the sum of these being substantially 100%.

The blends of the invention usually contain in total at least 70% of saturates, such as 70-98% or 70-90% or 90-98%.

If desired and especially for aviation gasoline, the blends may contain a hydrocarbon component which is a saturated aliphatic hydrocarbon of 4-6 carbons and which has a boiling point of less than 80°C under atmospheric pressure, such as 20-50°C, and especially is itself of Motor Octane Number greater than 88 in particular at least 90 e.g. 88-93 or 90-92. Examples of the hydrocarbon component include alkanes of 4 or 5 carbons in particular iso-pentane, which may be substantially pure or crude hydrocarbon fraction from reformate or isomerate containing at least 30% e.g. 30-80% such as 50-70%, the main contaminant being up to 40% mono methyl pentanes and up to 50% dimethyl butanes. The hydrocarbon component may be an alkane of boiling point (at atmospheric pressure) -20°C to +20°C e.g. n and/or iso butane optionally in blends with the C₅ alkane of 99.5:0.5 to 0.5:99.5, e.g. 88:12 to 75:25. n Butane alone or mixed with isopentane is preferred, especially in the above proportions, and in particular with a volume amount of butane in the composition of up to 20% such as 1-15% e.g. 1-8, 3-8 or 8-15%, especially 1-3.5%.

The hydrocarbon component boiling less than 80°C, in particular isopentane, may also be present in compositions of the invention which contain at least one compound A or A¹, of at least 10 carbon atoms, in particular those boiling at 160°C or above, such as A1, and A12-14. Relative amounts of these compounds A or A¹ to the low boiling component e.g. isopentane, may be 1-9:9-1 such as 5-9:5-1, especially with less than 20% of A or A¹ in the composition.

Cycloaliphatic hydrocarbons e.g. of 5-7 carbons such as cyclopentane or cyclohexane may be present but usually in amounts of less than 15% of the total e.g. 1-10%.

The compositions of the invention also preferably contain as component (d) at least one olefin, (in particular with one double bond per molecule) which is a liquid alkene of 5-10 e.g. 6-8 carbons, such as a linear or branched alkene e.g. pentene, isopentene hexene, isohexene or heptene or 2 methyl 2 pentene, or a mixture comprising alkenes which may be made by cracking e.g. catalytically or thermally cracking a residue from crude oil, e.g. atmospheric or vacuum residue; the mixture may be heavy or light catalytically cracked spirit (or a mixture thereof). The cracking may be steam assisted. Other examples of olefin containing mixtures are "C6 bisomer", catalytic polymerate, and dimate. The olefinic mixtures usually contain at least 10% w/w olefins, such as at least 40% such as 40-80% w/w. Preferred mixtures are (xi) steam cracked spirit (xii) catalytically cracked spirit (xiii) C6 bisomer and (xiv) catalytic polymerate, though the optionally cracked catalytically spirits are most advantageous. Amounts in the total composition of the olefinic mixtures especially the sum of (xi) - (xiv) (if any present) maybe 0-55, e.g. 10-55 or 18-37 such as 23-35 or 20-55 such as 40-55% Amounts of (xi) and (xii) (if present) in total in the composition are preferably 18-55, such as 18-35, 18-30 or 35-55% (by volume).

The olefin or mixture of olefins usually has an MON value of 70-90, usually a RON value of 85-95 and a ROAD value of 80-92.

The volume amount of olefin(s) in total in the gasoline composition of the invention may be 0% or 0-30%, e.g. 0.1-30% such as 1-30% in particular 2-25 e.g. 2-14% (especially 3-10). Usually the composition contains at least 1% olefin and a maximum of 18% or especially a maximum of 14%, but may be substantially free of olefin.

The compositions may also contain as component (e) at least one aromatic compound, preferably an alkyl aromatic compound such as toluene or o, m, or p xylene or a mixture thereof or a trimethyl benzene. The aromatics may have been added as single compounds e.g. toluene, or may be added as an aromatics mixture containing at least 30% w/w aromatic compounds such as 30-100% especially 50-90%. Such mixtures may be made from catalytically reformed or cracked gasoline obtained from heavy naphtha. Example of such mixtures are (xxi) catalytic reformate and (xxii) heavy reformate or heavy steam cracked spirit. Amounts of the single compounds e.g. toluene in the composition may be 0-35%, such as 2-33% e.g. 10-33%, while amounts of the aromatics mixtures especially the total of the reformates (xxi) & (xxii) (if any) in the composition may be 0-50%, such as 1-33% e.g. 2-15% or 2-10% or 15-32% v/v, and total amount of reformates (xxi), (xxii) and added single compounds (e.g. toluene) may be 0-50% e.g. 0.5-20% or 5-40, such as 15-35 or 5-25% v/v.

The aromatics usually have a MON value of 90-110 e.g. 100-110 and a RON value of 100-120 such as 110-120 and a ROAD value of 95-110. The volume amount of aromatic compounds in the composition is usually 0% or 0-50% such as less than 40% or less than 28% or less than 20% such as 1-50%, 2-40%, 3-28%, 4-25%, 5-20% (especially 10-20%), 4-10% or 20-35% especially of toluene. The gasoline composition may also be substantially free of aromatic compound. Amounts of aromatic compounds of less than 42%, e.g. less than 35% or especially less than 30% or 18% are preferred. Preferably the amount of benzene is less than 5% preferably less than 1.5% or 1% e.g. 0.1-1% of the total volume or less than 0.1% of the total weight of the composition.

The compositions may also contain as component (f) at least one oxygenate octane booster, usually of Motor Octane Number of at least 96-105 e.g. 98-103. The oxygenate may be any organic liquid molecule containing and preferably consisting of, CH and at least one oxygen atom e.g. 1-5 of bp less than 225°C. The octane booster is usually an ether e.g. a dialkyl ether, in particular an asymmetric one, preferably wherein each alkyl has 1-6 carbons, in particular one alkyl being a branched chain alkyl of 3-6 carbons in particular a tertiary alkyl especially of 4-6 carbons such as tert-butyl or tert-amyl, and with the other alkyl being of 1-6 e.g. 1-3 carbons, especially linear, such as methyl or ethyl. Examples of such oxygenates include methyl tertiary butyl ether (MTBE), ethyl tertiary butyl ether and methyl tertiary amyl ether. The oxygenate may also be a cyclic ether, in particular with 5 or 6 ring atoms in the or each ring, such as furan or tetrahydrofuran and its lower alkyl e.g. methyl derivatives. The oxygenate may also be an alcohol of 1-6 carbons e.g. ethanol. The oxygenate may also be an organic carbonate e.g. a dialkyl carbonate with 1-3 carbon atoms in each alkyl e.g. dimethyl carbonate.

The volume amount of the oxygenate may be 0 or 0-25% such as 1-25%, 2-20%, 2-10% or 5-20% especially 5-15%, but advantageously less than 3% such as 1-3% (especially of MTBE and/or ethanol). The oxygenate may also be substantially absent from the composition or gasoline of the invention, which is thus a substantially hydrocarbon fuel.

The present invention also provides a formulated unleaded gasoline comprising a blend composition of the invention comprising component (a) and (b) and at least one gasoline additive, e.g. as described above, in particular with the gasoline comprising less than 5%, e.g. less than 4% of triptane or 223 trimethyl pentane.

The blend of the invention contains at least one component (a) and component (b) and, (optionally (c) to (f), as well, and the formulated unleaded gasoline also contains at least one gasoline additive e.g. a motor gasoline or aviation gasoline additive, for example as listed in ASTM D-4814 the contents of which is herein incorporated by reference or specified by a regulatory body, e.g. US California Air Resources Board (CARB) or Environmental Protection Agency (EPA). These additives are distinct from the liquid fuel ingredients, such as MTBE. Such additives may be the lead free ones described in Gasoline and Diesel Fuel Additives, K Owen, Publ. By J.Wiley, Chichester, UK, 1989, Chapters 1 and 2, USP 3955938, EP 0233250 or EP 288296, the contents of which are herein incorporated by reference. The additives maybe pre-combustion or combustion additives. Examples of additives arc anti-oxidants, such as one of the amino or phenolic type, corrosion inhibitors, anti-icing additives e.g. glycol ethers or alcohols, engine detergent additives such as ones of the succinic acid imide, polyalkylene amine or polyether amine type and anti-static additives such as ampholytic surface active agents, metal deactivators, such as one of thioamide type, surface ignition inhibitors such as organic phosphorus compounds, combustion improvers such as alkali metal salts and alkaline earth metal salts of organic acids or sulphuric acid monoesters of higher alcohols, anti valve seat recession additives such as alkali metal compounds, e.g. sodium or potassium salts such as borates or carboxylates e.g. sulpho succinates, and colouring agents, such as azodyes. One or more additives (e.g. 2-4) of the same or different types may be used, especially combinations of at least one antioxidant and at least one detergent additive. Antioxidants such as one or more hindered phenols e.g. ones with a tertiary butyl group in one or both ortho positions to the phenolic hydroxyl group are preferred in particular as described in Ex.1 hereafter. In particular the additives may be present in the composition in amounts of 0.1-1 00ppm e.g. 1-20ppm of each, usually of an antioxidant especially one or more hindered phenols. Total amounts of additive are usually not more than 1000ppm e.g. 1-1000ppm.

The compositions and gasolines are free of organolead compounds, and usually of manganese additives such as manganese carbonyls.

The compositions and gasolines may contain up to 0.1% sulphur, e.g. 0.000-0.02% such as 0.002-0.01%w/w.

The gasoline compositions of the invention usually have a MON value of 80 to 105 such as 85-105, 85-90, 90-105 or 93-105 e.g. but especially 94-102. The RON value is usually 90-115 e.g. 102-115 such as 98-112 or 105-112, or 93-98 e.g. 94.5-97.5, or 97-101 while the ROAD value is usually 85-110 or 85-107 e.g. 98-106 or 102-108 or 85-95. Preferred gasoline compositions have MON 83-93, RON 93-98 and ROAD 85-95 or MON 85-90, RON 94-101 and ROAD 89-96 but especially MON 93-98, RON 102-108, ROAD 98-106, or MON 95-105, RON 102-115 e.g. 108-115 and ROAD 98-106. The Net calorific value of the gasoline (also called the Specific Energy) is usually at least 41.9 MJ/kg (18000 Btu/Ib) e.g. at least 43.0, 43.5 or 44.0 MJ/kg (18500, 18700 or 18,900 Btu/lb) such as 43.0-45.4 MJ/kg (18500-19500 Btu/lb), such as 43.5 - 44.9 or 44.0 - 44.7 MJ/kg (18700-19300 or 18900-19200 Btu/lb); the calorific value may be at least 42MJ/kg e.g. at least 43.5 MJ/kg such as 42-45 or 43-45 such as 43.5-44.5MJ/kg. The gasoline usually has a boiling range (ASTM D86) of 20-225°C, in particular with at most 5% e.g. 0-5% or 1-3% boiling in the range 161-200°C. The gasoline is usually such that at 70°C at least 10% is evaporated while 50% is evaporated on reaching a temperature in the range 77-120°C preferably 77-116°C and by 185°C, a minimum of 90% is evaporated. The gasoline is also usually such that 8-50% e.g. 10-40% may be evaporated at 70°C, 40-74% at 100°C, 70-99.5% at 150°C and 90-100% may be evaporated at 180°C; preferably 46-65% has been evaporated by 100°C. The Reid Vapour Pressure of the gasoline at 37.8°C measured according to ASTM D323 is usually 30-120, e.g. 40-100 such as 61-80 or preferably 50-80, 40-65, e.g. 45-65, 40-60 or 40-50Kpa. Especially the gasoline or blend has RON value of 90-115, MON value of 85-105, aromatics content of less than 35%, olefins content of less than 14%, benzene less than 1%, % evaporated at 70°C 10-40%, % evaporated at 100°C 40-74%, % evaporated at 150°C 70-99.5% and RVP of 40-60 kPa.

The gasoline compositions, when free of any oxygenates usually have a H:C atom ratio of at least 1.8:1 e.g. at least 2.0:1 or at least 2.1 or 2.2:1, such as 1.8-2.3:1 or 2.0-2.2:1. Advantageously the gasoline composition meets the following criteria. $Atom H : C \times [ 1 + oxy ] \times \left[\frac{Net Heat of Combustion + ROAD}{200}\right] \geq y ,$
wherein Atom H:C is the fraction of hydrogen to carbon in the hydrocarbons in the composition, oxy means the molar fraction of oxygenate, if any in the composition, Net Heat of Combustion is the energy derived from burning 11b (454g) weight of fuel (in gaseous form) in oxygen to give gaseous water and carbon dioxide expressed in Btu/1b units [MJ/kg times 430.35], and y is at least 350, 380, 410 or 430, in particular 350-440 e.g. 380-420 especially 400-420.

Among preferred blends of the invention are unleaded blends comprising as component (a) at least 5 or 10% of at least one individual compound A or A¹ and component (b) as defined above, with the proviso that when the compound A or A¹ is an alkane of 9 or 10 carbon atoms, then blend contains at least 10% of an alkane of 6 or 7 carbons of MON at least 70 and RON at least 90, and preferably contains less than 5% in total of 2,2,3-trimethyl pentane and 2,2,3-trimethyl butane.

Preferred formulated unleaded gasolines of the invention comprise at least one gasoline additive and the preferred unleaded blend above, with the proviso when the compound A or A¹ is an alkane of 9 or 10 carbon atoms, the blend preferably contains less than 5% in total of 2,2,3-trimethyl pentane and 2,2,3-trimethyl butane.

Preferred blends and gasolines of the invention can have MON values of 94-105 (e.g. 97-105), RON values of 103-115 (e.g. 107-115), ROAD values of 98-110 (e.g. 102-110), compound A or A¹ contents of 30-60% e.g. 40-60% (comprising 1 or 2 compounds A or A¹ especially A1 and/or A2), total naphtha contents of 35-65% (e.g. 35-55%) and 1-5% butane, the blends containing 1-8% e.g. 2-6% aromatics, 0-1% olefins and 91-99% (e.g. 94-98%) saturates. These are substantially aliphatic blends and gasolines of very high octane numbers, without the use of oxygenates such as MTBE, and also substantially saturated.

Other very high octane blends and gasolines of the invention can have MON values of 94-102 e.g. 94-99, RON values of 105-115, ROAD values of 99-107, compound A or A¹ contents of 30-60% e.g. 30-50% (comprising 1 or 2 compounds A or A¹ especially A1 and/or A2), medium naphtha contents of 5-30% and contents of total olefinic fraction such as steam cracked spirit of 30-50% and 1-5% butane, the blends containing 10-25% aromatics e.g. 12-18% aromatics, 4-14% olefins e.g. 6-12%, and 60-90% such as 70-80% saturates. These high octane materials are obtained without the use of oxygenates.

Further blends and gasolines of the invention can have MON values of 84-90, RON values of 93-98, ROAD values of 86-94, and contain compound A or A¹ in amount of 15-35% (especially of A2), total naphtha of 40-65% and olefinic fractions such as steam cracked spirit of 15-45% and 0 or 1-5% butane, with aromatic contents of 5-25% such as 10-18% olefin contents of 2-14% and saturate contents of 70-90%.

Other blends and gasolines of the invention can contain 10-35% compound A or A¹ (especially A2), and naphtha 30-50%, hydrocrackate 10-30% alkylate and/or isomerate 2-10%, and reformate 3-12%.

Other blends and gasolines of the invention can contain 10-35% compound A or A¹ (especially A2) and 3-12% reformate, 1-20% light naphtha/straight run gasoline, as well as alkylate and isomerate, the blend and gasoline preferably containing at least 70% of saturates.

The invention can provide motor gasolines, in particular of 91, 95, 97, 98 and 110 RON values, with desired high Octane Levels but low emission values on combustion in particular of at least one of total hydrocarbons, NOx, carbon monoxide, and carbon dioxide, especially of both total hydrocarbons and carbon dioxide. Thus the invention also provides the use of a compound A particularly A1 or A2 in unleaded gasoline of MON at least 80 e.g. 80 to less than 98, e.g. as an additive to or component therein, to reduce the emission levels on combustion, especially of at least one of total hydrocarbons, NOx, carbon monoxide and carbon dioxide especially both of total hydrocarbons and carbon dioxide. The invention also provides a method of reducing emissions of exhaust gases in the combustion of unleaded gasoline fuels of MON of at least 80 which comprises having at least 10% component (a), in particular A1 or A2, present in the fuel which is a gasoline of the invention. The invention also provides use of an unleaded gasoline of the invention in a spark ignition combustion engine to reduce emissions of exhaust gases. In the compositions, gasolines, methods and uses of the invention the component (a) is preferably used in an emission-reducing effective amount. The compositions of the invention may be used in supercharged or turbocharged engines, or in normally aspirated ones. The compound A, preferably A1 or A2, can reduce one or more of the above emission levels better than a mixture of aromatics and oxygenate at similar Octane Number and usually decrease the fuel consumption as well.

The gasolines of the invention may be used in internal combustion spark ignition engines. They may be used to power moving vehicles on land and/or sea and/or in the air; the invention also provides a method of moving such vehicles by combustion of a gasoline of the invention. The vehicle usually has a driver and especially means to carry at least one passenger and/or freight.

The engine sizes for motor gasoline use are usually at least 45cc e.g. 45-10000cc e.g. at least 200cc, such as 500-10000cc, in particular 950-2550, such as 950-1550, or 1250-1850cc, or 2500-10000cc such as 2500-5000 or 5000-9000cc. The engines have at least 1 cylinder, but preferably at least 2 or 3 cylinders, e.g. 3-16, especially 4-6 or 8 cylinders; each cylinder is usually of 45-1250cc e.g. 200-1200cc, in particular 240-520cc or 500-1000cc. The engines may be 2 stroke engines, but are preferably 4 stroke. Rotary engines e.g. of the Wankel type may be used. The motor engines may be used to power vehicles with at least 2 wheels e.g. 2-4 powered wheels, such as motor bicycles, tricycles, and 3 wheeled cars, vans and motor cars, in particular those vehicles legislated for use on a public highway but also off road e.g. 4 wheeled drive vehicles, sports cars for highway use, and racing cars, including drag racing cars and track racing cars. Power from the engine will preferably be connected to the driving wheels via a gearbox and clutch system, or other form of drive train system, to achieve the transition from a stationary to a mobile state. The engine and drive train will best allow a range of actual vehicle road speed of between 1-350km/h, preferably between 5-130km/h and allow for continuous variation of speed thereof. The road speed of the vehicle is usually reduced by a braking mechanism fitted to the vehicle, the braking being generally applied by friction. The engine may either by air or water cooled, the air motion induced by a moving vehicle being used to directly, or indirectly cool the engine. The vehicle comprises a means to facilitate a change of vehicle direction, e.g. a steering wheel or stick. Usually at least 10% of the vehicle distance travelled is carried out at greater than 5km/h.

The engines using aviation gasoline are usually in piston driven aircraft, i.e. with at least one engine driving a means for mechanically moving air such as at least one propeller. Each engine usually drives at least one propeller driving shaft with 1 or 2 propellors. The aircraft may have 1-10 propellers e.g. 2-4. The aircraft engines usually have at least 2 cylinders, e.g. 2 to 28 cylinders, each of which is preferably greater than 700cc in volume, such as 700-2000cc e.g. 1310cc. The total engine size is usually 3700-50000cc e.g. 3700 to 12000cc for single or twin engined passenger light aircraft, 12000 to 45000cc for 2 or 4 engined freight or airline use (e.g. 15-200 passengers, such as 50 to 150 passengers). The engines may have an engine power to weight ratio of at least 0.3Hp/lb wt of engine, e.g. 0.3-2Hp/lb, and may have a power to cylinder volume of at least 0.5 (Hp/cu.in) e.g. 0.5-2. Cylinders may be arranged in rows, V formation, H formation, flat ('horizontally opposed') or radially around a common propeller drive shaft. One or more rows/circles of cylinders may be used, e.g. flat 2, flat 4, flat 6, V12, 1 2 or 3 circles of 7 cylinders etc. Every cylinder has one and more preferably at least two spark plugs. A gear system may optionally be used to drive the propeller and or a supercharger Alternatively, an exhaust turbo charger may also be present. Exhaust outlets may be individual or run into a common manifold and preferably point in the opposite direction to forward flight. Fins may be present on the exterior of the engine for air cooling. Greater than 90% of the distance travelled by the engine, when in use, is usually spent at 500 feet or more above ground level. Typically, during greater than 90% of the time when the engine is running, the engine operates at above 1000rpm e.g. between 1000 to 3500 rpm.

The aircraft usually has at least one tank having a capacity of at least 1001, especially with a total capacity of at least 10001. Small and micro-light aircraft may have tanks substantially smaller in capacity but can operate on the unleaded gasoline described.

The gasolines of the invention may be made in a refinery by blending the ingredients to produce at least 200,0001/day of gasoline such as 1-10million 1/day. The gasoline may be distributed to a plurality of retail outlets for motor gasoline, optionally via wholesale or bulk outlets e.g. holding tanks, such as ones of at least 2 million I capacity e.g. 5-15 million 1. The distribution may be by pipeline or in tanks transported by road, rail or water, the tanks being of at least 50001 capacity. At the retail sites e.g. filling station, the motor gasoline is dispensed to a plurality of users, i.e. the drivers of the vehicles, e.g. at a rate of at least 100 or 1000 different users per day. For aviation use, the gasoline is usually made in a refinery to produce at least 1000 barrels per day (or 100,0001/day) such as 0.1-2 million 1/day. The avgas is usually distributed by tanker by road, rail or water, or pipelines directly to the airport distribution or holding tanks, e.g. of at least 300,0001 capacity, from whence it is distributed by pipeline or tanker (e.g. a mobile refuelling bowser to fuel a plurality of aircraft, e.g. at least 5/day per tank; the aircraft may have one or more on-board tank each of at least 1001 capacity.

The present invention is illustrated in the following Examples.

### Examples 1-7

Various unleaded blends are made up with compound A1 and/or A2 and various refinery streams as shown in Table 1.

7 Formulated gasolines are made, each containing one of the above blends and a 15mg/l of a phenolic antioxidant 55% minimum 2,4 dimethyl-6-tertiary butyl phenol 15% minimum 4 methyl-2, 6-ditertiary-butyl phenol with the remainder as a mixture of monomethyl and dimethyl-tertiary butyl phenols.

In each case the gasolines are tested for MON and RON, and their Reid Vapour Pressure at 37.8°C. The results are shown in table 1, which also shows their analyses and distillation profile (according to ASTM D86).

### Example 8

The emission characteristics on combustion of the formulated gasolines of Ex.1-7 are determined.

The fuels are tested in a single cylinder research engine at a speed/load of 50/14.3rps/Nm with a LAMBDA setting of 1.01, and the ignition setting is optimised for the comparative blend. The emissions of CO, CO₂ total hydrocarbons, Nox, are measured from the exhaust gases. The results are averaged and show a reduction in the emissions compared to a standard unleaded fuel.

### Example 9 and Comparative Ex. A

An unleaded blend was made up with 22446 pentamethyl heptane, blended with various refinery streams as shown in Table 3. Comp Ex. A, with heavy reformate meets the Europe 2005 requirement for high octane fuel with RON 97.0, MON 86.3 RVP at 37.8°C 54.7 kPa distillation profile according to ASTM D86, 10% evap, at 52.9°C 50% at 107.0°C and 90% at 166.1°C.

2 formulated gasolines were made, each containing one of the above blends and 15mg/l of the phenolic antioxidant used in Ex.1-7.

In each case the gasolines were analysed. The results are shown in table 3.

The emission characteristics on combustion of the formulated gasolines of Ex. 9 and Comp. A were determined.

The fuels were tested as in Ex. 1-7 in a single cylinder research engine at a speed/load of 20/7/2rps/Nm with LAMBDA setting of 1.01, and the ignition setting was optimised for the comparative blend A. The emissions of CO, CO₂ total carbon oxides, total hydrocarbons, NOₓ were measured from the exhaust gases as was the Fuel Consumption (expressed in g/h¹Whr). The results were averaged and compared to the comparative Ex.A. The degrees of change were as given in Table 4.

**Table 3**

| | Comp A | 8 |
|---|---|---|
| | Base Fuel | |
| Formulation % v/v | | |
| Butane | 3 | 3 |
| Full range catalytically cracked spirit | 20 | 20 |
| Alkylate | 40 | 40 |
| Light hydrocracked spirit | 7 | 7 |
| Full range steam cracked spirit | 10 | 10 |
| Heavy reformate | 20 | |
| 2,2,4,4,6-Pentamethylheptane | | 20 |
| Density kg/l | 0.7487 | 0.7264 |
| C:H | 1 : 1.889 | 1 : 2.076 |
| C% w/w | 86.4 | 85.25 |
| H% w/w | 13.6 | 14.75 |
| Benzene % v/v | 0.6 | 0.6 |
| Aromatics % v/v | 29.4 | 9.4 |
| Olefins % v/v | 9.0 | 9.0 |

**Table 4**

| **Example** | **CO** | **CO2** | **COx** | **THC** | **NOx** | **Fuel Economy** |
|---|---|---|---|---|---|---|
| | | | | | | |
| **Comp A** | 0% | 0.0% | 0.0% | 0.0% | 0.0% | 0.0% |
| **9** | -1.7% | -2.7% | -2.7% | 3.1% | -4.5% | 0.1% |

Figures denote % change relative to base (Fuel (Comp.A)

**Table 1**

| **Ex.** | **1** | **2** | **3** | **4** | **5** | **6** | **7** |
|---|---|---|---|---|---|---|---|
| Butane | 47 | 36 | 54 | 28 | 2.9 | | |
| cpd A2 | 20.0 | 10.0 | 49.2 | 28.0 | 41.6 | 24.1 | 20.4 |
| cpd A1 | 27.2 | 26.4 | 4.7 | - | - | | |
| Med Naphtha | 7.4 | 0.07 | 27.3 | 48.0 | 17.9 | | 23.7 |
| Light Naphtha | 43.2 | 60.6 | 13.6 | 1.5 | - | 41.1 | 35.4 |
| Hydrocrackate | | | | | | 21.5 | |
| Reformate | | | | | | 7.8 | |
| Alkylate | | | | | | 5.6 | |
| Steam Crack Spirit | | | | 19.7 | 37.6 | | 20.4 |
| | | | | | | | |
| % Aromatics | 4.0 | 4.7 | 3.6 | 11.6 | 15.2 | | 12.3 |
| % Olefins | 0.2 | 0.2 | 0.1 | 5.2 | 9.7 | | 5.5 |
| % Saturates | 95.8 | 95.1 | 96.3 | 83.2 | 75.1 | | 82.2 |
| | | | | | | | |
| RON | 110.0 | 104.5 | 110.0 | 95.0 | 110.0 | | 95.0 |
| MON | 100.0 | 95.5 | 100.0 | 86.0 | 96.9 | | 86.0 |
| RVP.kPa | 50.0 | 60.0 | 50.0 | 50.0 | 50.0 | | 52.3 |
| ROAD | 105 | 100 | 105 | 90.5 | 103.45 | | 90.5 |
| E70% v/v | 22.8 | 33.4 | 10.5 | 16.7 | 19.0 | | 31.4 |
| E100% v/v | 49.9 | 60.0 | 49.0 | 49.0 | 51.1 | | 53.5 |
| E150% v/v | 78.0 | 78.0 | 99.0 | 96.9 | 99.0 | | 78.0 |
| E180% v/v | 92.8 | 92.6 | 100.0 | 99.8 | 100.0 | | 93.2 |
| Benzene % v/v | 0.3 | 0.03 | 0.3 | 0.12 | 0.23 | | 0.12 |
| Sulphur % w/v | | | | 0.0005 | 0.0005 | | 0.0004 |

### Example 10

An unleaded blend was made up with 2,2,3,3-tetramethyl butane (12%), alkylate (45%), reformate (6%), isomerate (20%) and naphtha i.e. a straight sum gasoline (17%). The tetramethyl butane contained 86.6%, 2,2,3,3-tetramethyl butane, 3.6% 2,2,4-trimethyl pentane 3.7%, cis 3 methyl hexene 2 and 6% unknown and high boilers. It was made substantially according to the procedure of Marker and Oakwood J. Amer. Chem. Soc. 1938, 60, 258.

The blend was mixed with 15mg/l of the phenolic antioxidant used in Ex. 1-3. The formulated gasoline was tested for MON and RON which were found to be 88.7 and 93.0 respectively, ROAD value 90.85.

## Claims

1. A formulated unleaded gasoline of MON at least 80 and RON of 90 - 115 which comprises at least one motor or aviation gasoline additive, and an unleaded blend composition having a Motor Octane Number (MON) of at least 81 and Research Octane Number (RON) of at least 91 which blend composition comprises :
component (a) ; a total of at least 15% by volume of the blend composition of at least one branched chain hydrocarbon compound A, there being a minimum of at least 10 % of at least one individual compound A, wherein compound A is an alkane of 8-12 carbon atoms with 4, 5 or 6 branches, which are methyl or ethyl and
a total of at least 20 % by volume of at least one component (b), which is at least one liquid hydrocarbon or mixture thereof of bp 60 - 160 °C having a MON value of at least 70 and RON value of at least 90.

2. A gasoline as claimed in claim 1 wherein in the at least one branched chain hydrocarbon, there is at least one pair of geminal methyl branches which are on the 2 position of the carbon backbone chain.

3. A gasoline as claimed in claim 2 wherein in the at least one branched chain hydrocarbon, there are two or three pairs of geminal branches, at least two pairs being on adjacent carbon atoms.

4. A gasoline according to claim 1 wherein in the at least one branched chain hydrocarbon, there are one, two or three pairs of geminal methyl branch substituents on a 4-6 carbon chain backbone, and if any ethyl CMe₂ structure is present, then there are two ethyl CMe₂ groups in the compound.

5. A gasoline according to claim 1 wherein in the at least one branched chain hydrocarbon, there is one geminal methyl branch grouping on the backbone chain and on one or both of the adjacent carbon atoms of the backbone chain there is one or two methyl or ethyl branches, especially one or two methyl branches.

6. A gasoline according to of claim 1 wherein in the at least one branched chain hydrocarbon there are one, two or three pairs of geminal methyl branches on the backbone chain and if there arc two or three geminal pairs then at least two pairs are on adjacent backbone carbon atoms and if there is only one geminal pair then they are on the 2 position of the backbone carbon chain and there is a methyl branch at least on the 3 position of the backbone carbon chain.

7. A gasoline according to claim 1 wherein the at least one branched chain hydrocarbon has two or three pairs of geminal methyl branches, at least two pairs being on adjacent carbon atoms and the compound having a symmetrical structure.

8. A gasoline according to claim 1 wherein the at least one branched chain hydrocarbon has a linear backbone chain of four or six carbon atoms and has four to six methyl branches, in at least one geminal group, especially in the absence of a 1,2 ethyl group in the backbone.

9. A gasoline according to claim 1 wherein the at least one branched chain hydrocarbon has a linear backbone of five or six carbon atoms and has four to six branches in at least one geminal group, with the proviso that if there are four methyl branches and the compound contains an ethyl CMe₂ group, then the compound contains two such ethyl CMe₂ groups.

10. A gasoline according to claim 1 wherein the at least one branched chain hydrocarbon has one, two, or three carbon atoms with geminal methyl branches and if there is only one such carbon atom with geminal methyl branches then there is one or two branches on a vicinal carbon atom to the geminal one and any ethyl -C- chain group in the backbone chain has five carbon atoms.

11. A gasoline according to claim 1 wherein the at least one branched chain hydrocarbon is an alkane with alkyl substituents on vicinal internal carbon atoms with a total of four, five or six carbon atoms in said substituents.

12. A gasoline as claimed in claim 1 wherein the at least one branched chain hydrocarbon has no branched groups other than methyl or ethyl.

13. A gasoline as claimed in claim 1 wherein the at least one branched chain hydrocarbon has a backbone chain of carbon atoms in which no n-propyl or n-butyl groups form part of the backbone chain.

14. A gasoline according to claim 1 wherein said hydrocarbon is at least one of 3,3,4,4 tetramethyl hexane, 2,2,3,3 tetramethyl butane, 2,2,3,3 tetramethyl pentane, 2,2,3,3,4 pentamethyl pentane, 2,2,3,4,4 pentamethyl pentane, 2,3,3,4 tetramethyl pentane, 2,2,3,4 tetramethyl pentane, 2,2,3,3,4,4 hexamethyl pentane and 2,2,4,4,6 pentamethyl heptane, especially at least one of 2,2,3,3-tetramethyl butane, 3,3,4,4-tetramethyl hexane and 2,2,3,3 tetramethyl pentane and must especially at least one of 2,2,3,3-tetramethyl butane and 3,3,4,4-tetramethyl hexane.

15. A gasoline as claimed in any one of claims 1 to 14 wherein the gasoline further comprises as component (d) at least one olefin, which is a liquid alkene of five to ten carbons.

16. A gasoline as claimed in any one of claims 1 to 15 wherein the gasoline further comprises as component (e) at least one aromatic compound.

17. A gasoline as claimed in claim 16 in which the amount of aromatic compounds is less than 42 %.

18. A gasoline as claimed in any one of the claims 1 to 17 wherein the gasoline further comprises as component (f) at least one oxygenate octane booster.

19. A gasoline as claimed in any one of claims 1 to 16 wherein the gasoline composition has RON value of 90-115, MON value of 85-105, aromatics content of less than 35%, olefins content of maximum 14%, benzene less than 1%, % evaporated at 70°C 10-40%, % evaporated at 100°C 40-74%, % evaporated at 150°C 70-99.5% and RVP of 40-60 kPa.

20. An unleaded gasoline according to any one of claims 1 to 19 in which when the branched chain hydrocarbon is an alkane of 9 or 10 carbon atoms, then the blend composition contains less than 5% in total of 2,2,3-trimethyl pentane and 2,2,3-trimethyl butane.

21. A gasoline as claimed in any one of claims 1 to 18 in which one or more gasoline additive is present and is selected from the group consisting of anti-oxidants of the amino or phenolic type, corrosion inhibitors, anti-icing additives which are glycol ethers or alcohols, engine detergent additives of the succinic acid imide, polyalkylene amine or polyether amine type and anti-static additives which are ampholytic surface active agents, metal deactivators of thioamide type, surface ignition inhibitors which are organic phosphorus compounds, combustion improvers which are alkali metal salts and alkaline earth metal salts of organic acids or sulphuric acid monoesters of higher alcohols, anti valve seat recession additives which are alkali metal compounds and are sodium or potassium salts of boratcs or carboxylates including sulpho succinates, and colouring agents which are azodyes.

22. A gasoline as claimed in claim 21 in which combinations of at least one antioxidant and at least one detergent additive are present.

23. A gasoline as claimed in claim 22 in which antioxidants such as one or more hindered phenols c.g. ones with a tertiary butyl group in one or both ortho positions to the phenolic hydroxyl group are present.

24. A method of reducing emissions of exhaust gases in the combustion of an unleaded gasoline fuel of MON at least 80 and RON of 90 - 115 which fuel is a formulated gasoline as claimed in any one of claims 1 to 23 which method comprises having present in said gasoline at least 10 % by volume of component (a).

25. Method according to claim 24 wherein the gasoline is an unleaded motor gasoline.

26. Method according to claim 24 wherein the gasoline is an unleaded aviation gasoline.

## Patentansprüche

1. Formulierter bleifreier Kraftstoff mit einem MOZ von mindestens 80 und einem ROZ von 90 - 115, der mindestens ein Motor- oder Flugkraftstoffadditiv, und eine bleifreie Mischzusammensetzung mit einer Motor-Oktanzahl (MOZ) von mindestens 81 und einer Research-Oktanzahl (ROZ) von mindestens 91 umfaßt, wobei die Mischzusammensetzung: Komponente (a) mit insgesamt mindestens 15 Vol.-% der Mischzusammensetzung von mindestens einer verzweigtkettigen Kohlenwasserstoffverbindung A, wobei mindestens 10 % von mindestens einer einzelnen Verbindung A vorhanden sind, wobei Verbindung A ein Alkan mit 8 - 12 Kohlenstoffatomen mit 4, 5 oder 6 Verzweigungen ist, die Methyl oder Ethyl sind, und insgesamt mindestens 20 Vol.-% von mindestens einer Komponente (b), die zumindest ein flüssiger Kohlenwasserstoff oder ein Gemisch davon mit einem Sp. von 60 - 160 °C mit einem MOZ-Wert von mindestens 70 und einem ROZ-Wert von mindestens 90 ist, umfaßt.

2. Kraftstoff nach Anspruch 1, wobei es in dem mindestens einen verzweigtkettigen Kohlenwasserstoff mindestens ein Paar geminaler Methylverzweigungen gibt, die sich an Position 2 der Kohlenstoffhauptkette befinden.

3. Kraftstoff nach Anspruch 2, wobei es in dem mindestens einen verzweigtkettigen Kohlenwasserstoff zwei oder drei Paare geminaler Verzweigungen gibt, von denen sich mindestens zwei Paare an nachbarständigen Kohlenstoffatomen befinden.

4. Kraftstoff nach Anspruch 1, wobei es in dem mindestens einen verzweigtkettigen Kohlenwasserstoff eines, zwei oder drei Paare geminaler Methylverzweigungssubstituenten an einer 4 - 6 Kohlenstoffhauptkette gibt und es bei einer Ethyl-CMe₂-Struktur zwei Ethyl-CMe₂-Gruppen in der Verbindung gibt.

5. Kraftstoff nach Anspruch 1, wobei es in dem mindestens einen verzweigtkettigen Kohlenwasserstoff eine geminale Methylverzweigungsgruppierung an der Hauptkette gibt, und an einem oder beiden der nachbarständigen Kohlenstoffatome der Hauptkette eine oder zwei Methyl- oder Ethylverzweigungen, speziell eine oder zwei Methylverzweigungen vorliegen.

6. Kraftstoff nach Anspruch 1, wobei es in dem mindestens einen verzweigtkettigen Kohlenwasserstoff eines, zwei oder drei Paare geminaler Methylverzweigungen an der Hauptkette gibt, und, wenn es zwei oder drei geminale Paare gibt, dann mindestens zwei Paare an nachbarständigen Hauptkettenkohlenstoffatomen vorliegen und, wenn es nur ein geminales Paar gibt, diese dann an Position 2 der Kohlenstoffhauptkette vorliegen und eine Methylverzweigung zumindest an Position 3 der Kohlenstoffhauptkette vorliegt.

7. Kraftstoff nach Anspruch 1, wobei der mindestens eine verzweigtkettige Kohlenwasserstoff zwei oder drei Paare geminaler Methylverzweigungen aufweist, von denen mindestens zwei Paare an nachbarständigen Kohlenstoffatomen vorliegen und die Verbindung eine symmetrische Struktur hat.

8. Kraftstoff nach Anspruch 1, wobei der mindestens eine verzweigtkettige Kohlenwasserstoff eine lineare Hauptkette mit vier bis sechs Kohlenstoffatomen und vier bis sechs Methylverzweigungen in mindestens einer geminalen Gruppe, insbesondere in Abwesenheit einer 1,2-Ethylgruppe in der Hauptkette aufweist.

9. Kraftstoff nach Anspruch 1, wobei der mindestens eine verzweigtkettige Kohlenwasserstoff eine lineare Hauptkette mit fünf oder sechs Kohlenstoffatomen und vier bis sechs Verzweigungen in mindestens einer geminalen Gruppe aufweist, mit der Maßgabe, daß, wenn vier Methylverzweigungen vorliegen und die Verbindung eine Ethyl-CMe₂-Gruppe aufweist, dann die Verbindung zwei solcher Ethyl-CMe₂-Gruppen aufweist.

10. Kraftstoff nach Anspruch 1, wobei der mindestens eine verzweigtkettige Kohlenwasserstoff ein, zwei oder drei Kohlenstoffatome mit geminalen Methylverzweigungen aufweist und, wenn nur ein solches Kohlenstoffatom mit geminalen Methylverzweigungen vorliegt, dann eine oder zwei Verzweigungen an einem zu dem geminalen Kohlenstoffatom nachbarständigen Kohlenstoffatom vorliegt, und die Ethyl-C-Kettengruppe in der Hauptkette fünf Kohlenstoffatome aufweist.

11. Kraftstoff nach Anspruch 1, wobei der mindestens eine verzweigtkettige Kohlenwasserstoff ein Alkan mit Alkylsubstituenten an nachbarständigen internen Kohlenstoffatomen mit insgesamt vier, fünf oder sechs Kohlenstoffatomen in den Substituenten ist.

12. Kraftstoff nach Anspruch 1, wobei der mindestens eine verzweigtkettige Kohlenwasserstoff keine anderen verzweigten Gruppen als Methyl oder Ethyl aufweist.

13. Kraftstoff nach Anspruch 1, wobei der mindestens eine verzweigtkettige Kohlenwasserstoff eine Kohlenstoffatomhauptkette aufweist, in der keine n-Propyl- oder n-Butylgruppen einen Teil der Hauptkette bilden.

14. Kraftstoff nach Anspruch 1, wobei der Kohlenwasserstoff mindestens einer von 3,3,4,4-Tetramethylhexan, 2,2,3,3-Tetramethylbutan, 2,2,3,3-Tetramethylpentan, 2,2,3,3,4-Pentamethylpentan, 2,2,3,4,4-Pentamethylpentan, 2,3,3,4-Tetramethylpentan, 2,2,3,4-Tetramethylpentan, 2,2,3,3,4,4-Hexamethylpentan und 2,2,4,4,6-Pentamethylheptan, speziell mindestens einer von 2,2,3,3-Tetramethylbutan, 3,3,4,4-Tetramethylhexan und 2,2,3,3-Tetramethylpentan und besonders bevorzugt mindestens einer von 2,2,3,3-Tetramethylbutan und 3,3,4,4-Tetramethylhexan ist.

15. Kraftstoff nach einem der Ansprüche 1 bis 14, wobei der Kraftstoff ferner als Komponente (d) mindestens ein Olefin, das ein flüssiges Alken mit fünf bis zehn Kohlenstoffen ist, umfaßt.

16. Kraftstoff nach einem der Ansprüche 1 bis 15, wobei der Kraftstoff ferner als Komponente (e) mindestens eine aromatische Verbindung umfaßt.

17. Kraftstoff nach Anspruch 16, worin die Menge an aromatischen Verbindungen kleiner ist als 42 %.

18. Kraftstoff nach einem der Ansprüche 1 bis 17, wobei der Kraftstoff ferner als Komponente (f) mindestens einen Oxygenat-Oktan-Booster umfaßt.

19. Kraftstoff nach einem der Ansprüche 1 bis 16, wobei die Kraftstoffzusammensetzung einen ROZ-Wert von 90 - 115, einen MOZ-Wert von 85 - 105, einen Gehalt an aromatischen Verbindungen von weniger als 35 %, einen Gehalt an Olefinen von maximal 14 %, weniger als 1 % Benzol, eine prozentuale Verdampfungsrate bei 70 °C von 10 - 40 %, eine prozentuale Verdampfungsrate bei 100 °C von 40 - 74 %, eine prozentuale Verdampfungsrate bei 150 °C von 70 - 99,5 % und einen RVP von 40 - 60 kPa aufweist.

20. Bleifreier Kraftstoff nach einem der Ansprüche 1 bis 19, worin, wenn der verzweigtkettige Kohlenwasserstoff ein Alkan mit 9 oder 10 Kohlenstoffatomen ist, dann die Mischzusammensetzung weniger als 5 % insgesamt an 2,2,3-Trimethylpentan und 2,2,3-Trimethylbutan enthält.

21. Kraftstoff nach einem der Ansprüche 1 bis 18, worin ein oder mehrere Kraftstoffadditive vorliegen und aus der Gruppe ausgewählt ist/sind, bestehend aus Antioxidationsmitteln vom Amino- oder Phenoltyp, Korrosionsinhibitoren, Vereisungsverhinderern, die Glykolether oder Alkohole sind, Motorreinigungsadditiven vom Bersteinsäureimid-, Polyalkylenamin- oder Polyetheramintyp und Antistatikadditiven, die ampholytische oberflächenaktive Mittel sind, Metalldesaktivatoren vom Thioamidtyp, Glühzündungsinhibitoren, die organische Phosphorverbindungen sind, Verbrennungsverbesserungsmitteln, die Alkalimetallsalze und Erdalkalimetallsalze von organischen Säuren oder Schwefelsäuremonoester höherer Alkohole sind, Additive gegen Ventilsitzrückgang, die Alkalimetallverbindungen und Natrium- oder Kaliumsalze von Boraten oder Carboxylaten sind, einschließlich Sulphosuccinaten, und Färbemitteln, wie Azofarbstoffen.

22. Kraftstoff nach Anspruch 21, worin Kombinationen aus mindestens einem Antioxidationsmittel und mindestens einem Reinigungsadditiv vorliegen.

23. Kraftstoff nach Anspruch 22, worin Antioxidationsmittel wie eines oder mehrere gehinderte Phenole, z. B. eines mit einer tertiären Butylgruppe in einer oder beiden orthoStellungen zu der phenolischen Hydroxylgruppe vorliegen.

24. Verfahren zur Verringerung von Emissionen von Abgasen bei der Verbrennung eines bleifreien Kraftstoffes mit einem MOZ von mindestens 80 und einem ROZ von 90 - 115, wobei der Treibstoff ein formulierter Kraftstoff nach einem der Ansprüche 1 bis 23 ist, wobei das Verfahren die Gegenwart von mindestens 10 Vol.-% von Komponente (a) in dem Kraftstoff umfaßt.

25. Verfahren nach Anspruch 24, worin der Kraftstoff ein bleifreier Motorkraftstoff ist.

26. Verfahren nach Anspruch 24, worin der Kraftstoff ein bleifreier Flugkraftstoff ist.

## Revendications

1. Essence sans plomb formulée d'indice d'octane moteur d'au moins 80 et d'indice d'octane recherche de 90 à 115, laquelle comprend au moins un additif d'essence automobile ou d'avion, et une composition de mélange sans plomb ayant un indice d'octane moteur (IOM) d'au moins 81 et un indice d'octane recherche (IOR) d'au moins 91, laquelle composition de mélange comprend :
un composant (a) : un total d'au moins 15 % en volume de la composition de mélange d'au moins un composé A de type hydrocarbure à chaîne ramifiée, ayant un minimum d'au moins 10 % d'au moins un composé individuel A, le composé A étant un alcane de 8 à 12 atomes de carbone avec 4, 5 ou 6 ramifications qui sont des groupes méthyle ou éthyle et un total d'au moins 20 % en volume d'au moins un composant (b), lequel est au moins un hydrocarbure liquide ou un mélange d'hydrocarbures de point d'ébullition allant de 60 à 160°C ayant une valeur d'IOM d'au moins 70 et une valeur d'IOR d'au moins 90.

2. Essence selon la revendication 1, dans laquelle dans le au moins un hydrocarbure à chaîne ramifiée, il y a au moins une paire de ramifications méthyle géminales en position 2 de la chaîne carbonée principale.

3. Essence selon la revendication 2, dans laquelle dans le au moins un hydrocarbure à chaîne ramifiée, il y a deux ou trois paires de ramifications géminales, au moins deux paires étant sur des atomes de carbone adjacents.

4. Essence selon la revendication 1, dans laquelle dans le au moins un hydrocarbure à chaîne ramifiée, il y a un, deux ou trois paires de substituants sous forme de ramifications méthyle géminales sur un chaîne principale ayant de 4 à 6 atomes de carbone, et si une quelconque structure éthylCMe₂ est présente, alors il y deux groupes éthylCMe₂ dans le composé.

5. Essence selon la revendication 1, dans laquelle dans le au moins un hydrocarbure à chaîne ramifiée, il y a un groupement sous forme de ramification méthyle géminale sur la chaîne principale et sur un ou les deux atomes de carbone adjacents de la chaîne principale, il y a une ou deux ramifications méthyle ou éthyle, plus spécifiquement une ou deux ramifications méthyle.

6. Essence selon la revendication 1, dans laquelle dans le au moins un hydrocarbure à chaîne ramifiée, il y a une, deux ou trois paires de ramifications méthyle géminales sur la chaîne principale et si il y a deux ou trois paires géminales alors au moins deux paires sont sur des atomes de carbone adjacents de la chaîne principale et si il y a seulement une paire géminale alors elle est en position 2 de la chaîne carbonée principale et il y a une ramification méthyle au moins en position 3 de la chaîne carbonée principale.

7. Essence selon la revendication 1, dans laquelle le au moins un hydrocarbure à chaîne ramifiée a deux ou trois paires de ramifications méthyle géminales, au moins deux paires étant sur des atomes de carbone adjacents et le composé ayant une structure symétrique.

8. Essence selon la revendication 1, dans laquelle le au moins un hydrocarbure à chaîne ramifiée a une chaîne principale linéaire de quatre ou six atomes de carbone et possède de quatre à six ramifications méthyle, dans au moins un groupe géminal, plus spécifiquement en l'absence d'un groupe éthyle en position 1 et 2 sur la chaîne principale.

9. Essence selon la revendication 1, dans laquelle le au moins un hydrocarbure à chaîne ramifiée a une chaîne principale linéaire de cinq ou six atomes de carbone et possède de quatre à six ramifications dans au moins un groupe géminal, à condition que si il y a quatre ramifications méthyle et que le composé contient un groupe éthylCMe₂, alors le composé contient deux de ces groupes éthylCMe₂.

10. Essence selon la revendication 1, dans laquelle le au moins un hydrocarbure à chaîne ramifiée a un, deux ou trois atomes de carbone avec des ramifications méthyle géminales et si il y a seulement un atome de carbone avec des ramifications méthyle géminales alors il y a une ou deux ramifications sur un atome de carbone vicinal par rapport au géminal et n'importe quel groupe à chaîne éthyl-C- dans la chaîne principale a cinq atomes de carbone.

11. Essence selon la revendication 1, dans laquelle le au moins un hydrocarbure à chaîne ramifiée est un alcane avec des substituants alkyle sur les atomes de carbone internes vicinaux avec un total de quatre, cinq ou six atomes de carbone dans lesdits substituants.

12. Essence selon la revendication 1, dans laquelle le au moins un hydrocarbure à chaîne ramifiée ne possède aucun groupe ramifié autre qu'un groupe méthyle ou éthyle.

13. Essence selon la revendication 1, dans laquelle le au moins un hydrocarbure à chaîne ramifiée a une chaîne principale d'atomes de carbone dans laquelle aucun groupe n-propyle ou n-butyle ne fait partie de la chaîne principale.

14. Essence selon la revendication 1, dans laquelle ledit hydrocarbure est au moins un parmi le 3,3,4,4-tétraméthylhexane, le 2,2,3,3-tétraméthylbutane, le 2,2,3,3-tétraméthylpentane, le 2,2,3,3,4-pentaméthylpentane, le 2,2,3,4,4-pentaméthylpentane, le 2,3,3,4-tétraméthylpentane, le 2,2,3,4-tétraméthylpentane, le 2,2,3,3,4,4-hexaméthylpentane et le 2,2,4,4,6-pentaméthylheptane, plus spécifiquement au moins un parmi le 2,2,3,3-tétraméthylbutane, le 3,3,4,4-tétraméthylhexane et le 2,2,3,3-tétraméthylpentane et de manière la plus spécifique au moins un parmi le 2,2,3,3-tétraméthylbutane et le 3,3,4,4-tétraméthylhexane.

15. Essence selon l'une quelconque des revendications 1 à 14, laquelle essence comprend en outre en tant que composant (d) au moins une oléfine, laquelle est un alcène liquide contenant de cinq à dix atomes de carbone.

16. Essence selon l'une quelconque des revendications 1 à 15, laquelle essence comprend en outre en tant que composant (e) au moins un composé aromatique.

17. Essence selon la revendication 16, dans laquelle la quantité des composés aromatiques est inférieure à 42 %.

18. Essence selon l'une quelconque des revendications 1 à 17, laquelle essence comprend en outre en tant que composant (f) au moins un booster d'indice d'octane oxygéné.

19. Essence selon l'une quelconque des revendications 1 à 16, dans laquelle la composition d'essence a une valeur d'IOR de 90 à 115, une valeur d'IOM de 85 à 105, une teneur en composés aromatiques inférieure à 35 %, une teneur maximale en oléfines de 14 %, une teneur en benzène inférieure à 1 %, un pourcentage d'évaporation à 70°C de 10 à 40 %, un pourcentage d'évaporation à 100°C de 40 à 74 %, un pourcentage d'évaporation à 150°C de 70 à 99,5 % et une tension de vapeur selon Reid (TVR) de 40 à 60 kPa

20. Essence sans plomb selon l'une quelconque des revendications 1 à 19 dans laquelle lorsque l'hydrocarbure à chaîne ramifiée est un alcane de 9 ou 10 atomes de carbone, alors la composition de mélange contient moins de 5 % au total de 2,2,3-triméthylpentane et de 2,2,3-triméthylbutane.

21. Essence selon l'une quelconque des revendications 1 à 18 dans laquelle un ou plusieurs additifs d'essence sont présents et sont choisis dans le groupe constitué par des antioxydants de type amino ou phénolique, des inhibiteurs de corrosion, des additifs anti-givrage qui sont des éthers de glycol ou des alcools, des additifs détersifs de moteur de type imide d'acide succinique, polyalkylèneamine et polyétheramine et des additifs antistatiques qui sont des agents tensioactifs ampholytes, des désactivateurs de métaux de type thioamide, des inhibiteurs d'auto-allumage par points chauds en surface qui sont des composés organophosphorés, des agents améliorant le combustion qui sont des sels de métaux alcalins et des sels de métaux alcalinoterreux d'acides organiques ou des monoesters de l'acide sulfurique d'alcools supérieurs, des additifs anti-récession de siège de soupape qui sont des composés à base d'un métal alcalin et sont des sels de sodium ou de potassium de borates ou de carboxylates comprenant des succinates, et des agents de coloration qui sont des colorants azoïques.

22. Essence selon la revendication 21 dans laquelle des combinaisons d'au moins un antioxydant et d'au moins un additif détersif sont présentes.

23. Essence selon la revendication 22 dans laquelle des antioxydants tels qu'un ou plusieurs phénols encombrés, par exemple, des phénols avec un groupe tert-butyle sur une position ortho ou sur les deux positions ortho du groupe hydroxyle phénolique, sont présents.

24. Procédé destiné à réduire les émissions des gaz d'échappement d'un carburant à base d'essence sans plomb d'IOM d'au moins 80 et d'IOR de 90 à 115, lequel carburant est une essence formulée selon l'une quelconque des revendications 1 à 23, lequel procédé comprend le fait d'avoir présent dans ladite essence au moins 10 % en volume de composant (a).

25. Procédé selon la revendication 24, dans lequel l'essence est une essence automobile sans plomb.

26. Procédé selon la revendication 24, dans lequel l'essence est une essence d'avion sans plomb.
